

July 22, 1952

C. J. STALEGO ET AL

2,603,833

## METHOD AND APPARATUS FOR FORMING FIBERS

Filed Dec. 30, 1948

2 SHEETS—SHEET 1



INVENTOR.  
Charles J. Stalego <sup>a</sup>  
BY Warren W. Drummond

*Staelin & Guerman*  
ATTORNEYS

July 22, 1952

C. J. STALEGO ET AL

2,603,833

METHOD AND APPARATUS FOR FORMING FIBERS

Filed Dec. 30, 1948

2 SHEETS—SHEET 2



INVENTOR.  
Charles J. Stalego <sup>2nd</sup>  
BY Warren W. Drummond

Stachin & Guernan  
ATTORNEYS

## UNITED STATES PATENT OFFICE

2,603,833

METHOD AND APPARATUS FOR FORMING  
FIBERS

Charles J. Stalego and Wendell W. Drummond,  
Newark, Ohio, assignors to Owens-Corning  
Fiberglas Corporation, Toledo, Ohio, a corpora-  
tion of Delaware

Application December 30, 1948, Serial No. 68,164

9 Claims. (Cl. 18—2.4)

## 1

This invention relates to an improved method and apparatus for producing fibers from glass or materials which become molten or soft when subjected to heat and which may be drawn out into fine fibers when in a softened state.

One of the objects of this invention is to provide a simple and economical process and apparatus for producing fibers which may be as fine as one micron or less in diameter from a body of heat softened glass or material having characteristics similar to glass.

Another object of this invention is to subject a body of heat softened material to the action of centrifugal force of sufficient magnitude to draw out the material and project the same into a blast of gas moving at a velocity high enough to further draw out the material into fine fibers. In accordance with this invention the blast is obtained by burning a combustible mixture of gases within a combustion chamber at pressures above atmospheric and by discharging the burned gases or products of combustion from the chamber through an outlet so proportioned with respect to the quantity of gas burned in the chamber that the burned gases are forced from the chamber at a velocity sufficient to attenuate heat softened glass into fibers.

Still another object of this invention is to heat the material or glass to a temperature above the softening point thereof by introducing the material directly into the burner combustion chamber during the interval the combustible mixture of gases is burning within the chamber and thereby eliminating the necessity of providing separate burners or heating devices for heating the material to the softening or attenuating temperature.

A further object of this invention is to rotate the bottom wall of the chamber on which the heat softened material collects at a speed determined to provide the centrifugal force required to flow the heat softened material radially outwardly through the burner chamber outlet and into the blast of burned gas issuing from the outlet.

A still further feature of this invention is to separate the heat softened material as it flows outwardly under the influence of the centrifugal force into a multiplicity of small streams or filaments which are projected by the action of the centrifugal force into the blast escaping through the burner outlet and are attenuated into fine fibers by the force of the blast.

Still another feature of this invention is to heat the glass to such a high temperature within the

## 2

burner that the glass issuing from the burner is in a very high fluid condition and is atomized or broken up into extremely fine particles by the action of centrifugal force and the blast of burned gases, and these particles are then attenuated into fine fibers as they cool in their high velocity motion.

The foregoing as well as other objects will be made more apparent as the description proceeds, especially when considered in connection with the accompanying drawings, wherein:

Figure 1 is a semi-diagrammatic longitudinal sectional view through one type of apparatus capable of carrying out the several steps of the process;

Figure 2 is a cross-sectional view taken on the line 2—2 of Figure 1;

Figure 3 is a cross-sectional view taken on the line 3—3 of Figure 1;

Figure 4 is a semi-diagrammatic longitudinal sectional view of a modified form of apparatus; and

Figure 5 is a diagrammatic sectional view similar to Figure 4 showing still another embodiment of this invention.

It will be apparent as this description proceeds that the process and apparatus disclosed herein may be successfully employed to produce fibers on a commercial basis from inorganic materials other than glass but having characteristics similar to glass. Such materials are of a nature which become soft when subjected to heat and are capable of being drawn out into fine fibers when in a softened condition. These properties are present in many different types of thermoplastic materials and are also found in various kinds of synthetic resins. However, the present invention has been particularly developed in connection with the manufacture of glass fibers and for this reason glass is referred to particularly in the following description.

The various steps of the process will perhaps be more fully understood by a description of one type of apparatus that may be employed for carrying out the steps of the process. With this in view, reference is made to the embodiment of the invention shown in Figures 1 to 3 inclusive of the drawings. In detail, the numeral 10 indicates a cylindrical burner having refractory side and end walls 11 and 12 respectively. The burner 10 is suitably supported in a vertical position and the end wall 12 forms the bottom of the burner. The refractory walls of the burner are enclosed in a suitable metal casing 13 and the latter is journaled in bearings 14 carried by suitable sup-

porting structure 15 in a manner to enable rotation of the burner about the vertical axis of the latter.

The refractory walls of the burner cooperate to form a combustion chamber 16 having the upper end closed by a top wall 17 which may also be formed of a refractory material and is preferably enclosed within the metal casing 13. The top wall 17 is formed with a centrally arranged opening 18 through which a supply tube 19 projects into the upper end of the combustion chamber 16. The supply tube is suitably secured to the top wall 17 and rotates as a unit with the burner 10. Cooperating with the top wall 17 of the burner to form a fuel mixture inlet chamber 20 is a ring 21 formed of a refractory material and secured in the burner at the top of the combustion chamber 16. The opening through the ring is of a diameter to receive the lower end of the supply tube 19 and the latter is suitably secured to the ring.

The selected fuel mixture is introduced into the chamber 20 through a plurality of ports 22 formed in the side wall of the burner adjacent the top of the latter and spaced equal distances from each other circumferentially of the burner. The ports 22 communicate with an annular manifold 23 fixed to the support 15 and connected to a source of fuel mixture by a conduit 24. It follows from the above that the burner 10 rotates relative to the fuel mixture supply manifold 23 and in order to prevent the escape of fuel mixture from the manifold suitable sealing means is provided between the adjacent surfaces of the manifold and burner. One type of seal that may be used for the above purpose is shown in Figure 1 of the drawings as comprising a pair of contracting sealing rings 25 respectively supported in annular grooves 26 formed in the inner surface of the annular manifold at opposite sides of the fuel supply chamber therein. These rings respectively frictionally engage the metal casing 13 at opposite sides of the ports 22 and thereby prevent the escape of fuel mixture flowing from the manifold 23 to the ports 22.

The fuel mixture employed may be ordinary natural gas or manufactured gas mixed with the proper amount of air by orthodox mixing equipment not shown herein. In any case, the combustible mixture of gases is introduced into the burner at pressures somewhat above atmospheric pressure and at a rate below the rate of flame propagation of the mixture in the atmosphere.

The combustible mixture of gases are admitted to the combustion chamber 16 through a multiplicity of passages 27 formed in the ring 21 and are ignited as they enter the chamber 16. The combustible mixture of gases burn within the confines of the chamber 16 to effect a very high rate of expansion and the resulting temperature heats the refractory walls of the chamber to a point where these walls become incandescent. The extremely high temperature of the refractory walls of the chamber 16 accelerates the rate of burning of the combustible mixture of gases substantially above the rate of flame propagation of the gas mixture in the atmosphere.

The burned gases or products of combustion are discharged from the combustion chamber 16 through a plurality of slots 28 formed in the side wall 11 of the burner at the bottom of the chamber 16 and spaced equal distances from each other circumferentially of the burner. The combined area of the slots or outlet openings 28 is so proportioned with respect to the quantity of fuel

mixture burned within the combustion chamber 16 that the burned gases are forced through the slots 28 in the form of a blast having a temperature which exceeds the softening temperature of glass and having a velocity sufficiently high to attenuate heat softened glass into fine fibers. In practice the combined area of the outlet openings 28 may be so proportioned with respect to the volume of the combustion chamber 16 to enable obtaining a gaseous blast having a temperature as high or higher than 3,000° F. and having a velocity as high or higher than 1,200 feet per second. Velocities in the order of 1,200 feet per second are of course substantially greater than the rate of flame propagation of the combustible mixture of gases in the atmosphere and provide ample force to reduce a body of glass of substantial size to fibers having diameters as small as one micron or less.

It will of course be understood that the combined area of the outlet openings 28 may be varied to some extent relative to the volume of the combustion chamber 16, depending upon the heat required in the blast issuing from the outlet openings. Outlet openings providing a greater area relative to the volume of the combustion chamber 16 permit burning a greater amount of gas and result in generating higher heat in the blast. However, this advantage is obtained at the expense of the velocity of the blast and for this reason the combined area of the outlet openings 28 is ordinarily no greater than necessary to obtain in the blast the heat required to raise or maintain the temperature of the glass to the desired attenuating temperature.

In accordance with the present invention the heat resulting from the high rate of combustion within the chamber 16 is employed to melt or soften a body of glass prior to reducing the latter to fine fibers. As shown particularly in Figure 1 of the drawings, glass is supplied into the combustion chamber 16 through the tube 19 from a tank or receptacle 29 diagrammatically shown as having an entrant conduit 30 and a discharge opening 31. The discharge opening 31 is formed in the bottom of the tank 29 and the latter is supported so that the opening 31 registers with the upper end of the supply tube 19. In the present instance the combustible mixture of gases is introduced into the tank 29 through the opening 30 and is burned in the space provided in the tank above the level of the glass. The combustible mixture of gases supplied to the tank 29 may be the same as the gas admitted to the burner 10 and is preferably burned in the tank 29 to provide a pressure on the glass which is sufficiently high to enable feeding the glass into the burner against the pressure existing in the combustion chamber 16.

It follows from the above that the supply of glass is heated in the tank 29 before being introduced into the combustion chamber 16. This initial heating of the glass within the tank 29 is not required, however, because the temperature available within the combustion chamber 16 is high enough to melt or soften the glass to the attenuating temperature. The chief purpose of burning the fuel mixture within the tank 29 is to supply the necessary pressure for feeding the glass into the combustion chamber against the pressure existing in the latter without cooling the glass. Other arrangements for feeding the glass may be resorted to, such for example as providing an extremely long supply tube leading from the tank 29 to the burner.

The molten or heat softened glass introduced into the combustion chamber 16 is deposited on the bottom wall 12 of the burner and this wall may be shaped to provide a well 32 for accommodating the heat softened glass. Referring again to Figure 1 of the drawings, it will be noted that the well is generally conical in shape with the apex in axial alignment with the burner and with the inner surfaces tapering outwardly to the discharge slots 18 in the side wall of the burner.

The burner 10 is rotated at a speed to provide the centrifugal force required to flow the molten or heat softened glass generally radially outwardly along the inner surface of the bottom wall 12 to the discharge slots 28. It is important to note that as the molten or heat softened glass flows radially outwardly over the bottom wall 12 any cords that may be present in the glass are stretched and thereby reduced in size. Thus the molten glass is mixed to some extent as it flows outwardly along the bottom wall 12 and the homogeneity of the glass is improved.

The centrifugal force resulting from rotation of the burner 10 is also sufficient to actually project the heat softened glass through the discharge slots 28 and into the blasts of burned gases issuing from the discharge slots. If desired, the heat softened glass may be separated into a multiplicity of individual streams of filaments by serrations 33 formed on the bottom edges of the discharge slots 28. As a result, relatively small streams of heat softened glass are projected into the blasts of burned gases discharging from the slots 28. This general arrangement provides in effect a two-phase attenuation of the heat softened glass, the first phase being accomplished by drawing out the heat softened glass under the influence of centrifugal force and the second phase being accomplished by the force of the burned gases contained within the blasts.

Any suitable means may be provided for rotating the burner 10 at the desired speed. In the present instance a pulley 34 is secured to the burner 10 adjacent the upper end of the latter and is supported on the support 15 through the medium of thrust bearings 35. This pulley is connected to a suitable prime mover, not shown herein, by a belt 36. The speed at which the burner 10 is rotated depends upon the viscosity of the glass deposited on the bottom wall 12 of the burner and also to some extent upon the size of fibers required. Assuming for the purpose of this disclosure that the diameter of the burner approximates twelve inches, speeds of between 500 and 1,000 R. P. M. are sufficient to produce the centrifugal force required to flow the heat softened glass radially outwardly into the blasts. It is to be understood, however, that the particular speeds noted above are not critical and may be varied considerably depending upon the viscosity of the glass deposited on the bottom wall 12 of the burner.

#### Operation

In use, glass or materials having characteristics similar to glass is introduced into the chamber 16 of the tube 19 and is deposited in the well 32 formed by the bottom wall 12 of the burner. As the glass or other material passes from the delivery end of the supply tube 19 to the well 32 it is heated by the burning gases within the combustion chamber 16 to a temperature sufficiently high to melt or substantially soften the glass or other material. During the above operation the burner 10 is rotated about the vertical axis of the combustion chamber 16 and the heat softened

material deposited on the inner surface of the well 32 flows radially outwardly under the influence of centrifugal force. As the heat softened material passes over the serrated surfaces 33 of the outlet slots 28 it is divided into a multiplicity of generally radially extending closely spaced streams. These streams are introduced directly into the burned gases or products of combustion flowing through the slots 28 so that the force of the gases coact with the centrifugal force acting on the heat softened material to draw out the streams and project the same into the blasts issuing from the slots 28. Thus regardless of the peripheral speed of the slotted portion of the burner, the individual streams are projected radially outwardly into the blasts and are further attenuated to form extremely fine fibers by the heat and force of the blasts.

Referring now to the embodiment of the invention shown in Figure 4 of the drawings, it will be noted that this construction differs from the apparatus previously described in two major respects. In the first place, the glass tank 29 is replaced by means for feeding glass forming material such as glass cullet or glass marbles directly into the combustion chamber 35 of the burner 36. In the second place, the burner 36 is fixed against rotation with the exception of the bottom wall 31 and the latter is supported for rotation about the vertical axis of the burner.

The means for introducing glass forming material such as batch, cullet or marbles into the combustion chamber 35 comprises a supply tube 38 similar to the tube 19 in that the lower end projects into the upper end of the combustion chamber 35 through the central opening formed in the ring 21. The upper end of the supply tube 38 is connected to a source of supply, not shown, for the glass forming material.

Inasmuch as the combustible mixture of gases in the chamber 35 burns under pressures somewhat above atmospheric, it may be necessary to provide a pressure lock within the tube 38. A suitable pressure lock is diagrammatically shown in Figure 4 and may be similar to the one disclosed in the Dockerty Patent 2,286,903. In any case, the purpose of the pressure lock is to prevent the burner chamber pressure from escaping through the supply tube 38 when glass forming material is fed to the combustion chamber. In general, the pressure lock comprises two slide valves 39 and 40 spaced from each other in the direction of length of the supply tube 38 and operable independently of one another. The arrangement is such that when it is desired to feed glass forming material into the burner the top valve 39 is closed and the bottom valve 40 is opened, enabling the material trapped between the two valves to drop by gravity into the combustion chamber 35.

As the glass forming material passes downwardly through the combustion chamber 35 it is heated to a sufficiently high temperature to form a body of glass and the latter is deposited in the well 41 formed by bottom wall 31 of the burner. The bottom wall 31 is formed separately from the side walls of the burner and cooperates with the bottom edges of the side burner walls to form an annular outlet opening 42 through which the products of combustion or burned gases escape from the chamber.

As in the first described form of the invention, the cross-sectional area of the annular outlet opening 42 is so proportioned with respect to the volume of the combustion chamber 35 that

burned gases are forced through the annular opening 42 in the form of a ring-like blast having a temperature exceeding the softening temperature of glass and having a velocity sufficiently high to attenuate the heat softened glass into fibers. The bottom wall 37 of the combustion chamber 35 is rotated about the vertical axis of the chamber at a speed determined to provide the centrifugal force required to flow heat softened glass generally radially outwardly along the inner surface of the wall 37 to the annular outlet opening 42. If desired, the top annular edge 43 of the bottom wall 37 may be serrated for the purpose of separating the heat softened glass into a multiplicity of individual streams before the glass is discharged through the outlet opening 42. As the heat softened glass flows outwardly over the peripheral edge of the bottom wall 37 into the annular outlet 42 it is subjected to the force of the burned gases or products of combustion escaping from the combustion chamber 35. Thus the heat softened glass is drawn through the annular outlet 42 by the blast of burned gases and is attenuated into fibers by the heat and force of this blast.

The bottom wall 37 is rotated at the desired speed by a vertical shaft 43 journaled in bearings 44 which in turn are secured to a fixed support 45. A pulley 46 is secured to the shaft between the bearings and is connected to a suitable prime mover 47 by a belt 48.

The modification shown in Figure 5 of the drawings illustrates a burner unit similar to the one featured in Figure 4 except that the bottom wall 49 is driven from a point above the burner and the incoming combustible mixture of gases is directed generally radially inwardly toward the vertical axis of the burner. Also, molten glass is supplied to the combustion chamber 50 from a tank 51 containing a body of molten glass and suitably supported directly above the burner.

In detail, the bottom wall 49 is connected at its center to the lower end of a vertical shaft 52 formed of a high heat resistant material, such for example as nickel, tungsten or platinum. This shaft projects upwardly through the combustion chamber 50 and through the tank 51 to a point substantially above the top wall of this tank. The upper end of the shaft is journaled in bearings 53 and is connected to a prime mover, not shown herein.

Surrounding the portion of the shaft 52 which extends through the bottom wall of the tank 51 is a cylinder 54 also formed of a high heat resistant metal, such for example as platinum. The upper end of the cylinder extends for some distance above the bottom wall of the tank so that molten glass within the tank flows over the top edge of the tube and passes downwardly along the inner surface of the tube into the combustion chamber. The molten glass flowing from the bottom of the cylinder 54 is forced inwardly against the shaft 52 by the pressure of the incoming fuel mixture and as a consequence the molten glass may be fed into the combustion chamber against the pressure which exists in this chamber.

The combustible mixture of gases is introduced into an annular manifold 55 through intake ports 56 and is discharged from the manifold radially inwardly toward the shaft 52 through a multiplicity of passages formed in the annular ring 57. The combustible mixture of gases flows

through the annular ring 57 under pressures above atmospheric and as a consequence the molten glass leaving the lower end of the cylinder 54 is directed inwardly against the shaft 52 to wet the latter. Thus the molten glass flows downwardly along the shaft 52 into the combustion chamber and is subjected to the high temperature of the burning gases within this chamber. The molten glass eventually is collected on the bottom wall 49 and flows outwardly under the influence of centrifugal force into the annular blast discharging from the circular outlet opening 58 which corresponds to the opening 42 described in connection with Figure 4. The operation of the embodiment shown in Figure 5 is generally the same as the operation previously described in connection with Figure 4.

We claim:

1. The process of making fibers from a heat softenable material which comprises burning a combustible mixture of gases within a substantially closed chamber and discharging the burned gases generally outwardly and radially from the chamber in the form of a blast moving at a velocity sufficient to attenuate the heat softened material into fibers, heating a body of the material to a softened state within said chamber, subjecting a body of said heat softened material to the action of centrifugal force to flow the heat softened material into the blast, and entraining the heat softened material in the blast whereby the material is carried away from the chamber by the blast and is attenuated into fibers by the heat and force of the blast.
2. The process of making fibers from a material capable of being softened by heat which comprises burning a combustible mixture of gases within a substantially closed chamber and discharging the burned gases from a restricted outlet in a wall of the chamber in the form of a substantially continuous annular blast moving at a velocity sufficient to attenuate heat softened material into fibers, heating a body of the material to a molten state within said chamber, subjecting the heat softened material to the action of centrifugal force to flow the heat softened material under the influence of the centrifugal force outwardly into the annular blast of the burned gases discharged from the chamber whereby the heat-softened material is carried away from the chamber by the blast, and attenuating the heat softened material into fibers by the heat and force of the blast.
3. The process of making glass fibers which comprises burning a combustible mixture of gases within a substantially closed chamber and discharging the burned gases through an opening in one side of the chamber adjacent the bottom wall of the latter in the form of a radially directed blast of a temperature above the attenuating temperature of glass and having a velocity sufficient to attenuate softened glass into fibers, heating a body of glass to a temperature which exceeds the softening point of glass by introducing the body of glass into the burning gases within the chamber, collecting the heat softened glass on the bottom wall of the chamber and subjecting the heat softened glass to the action of centrifugal force, flowing the heat softened glass under the influence of centrifugal force over the bottom wall of the chamber in an outward direction and into the burned gases discharged as a blast through the outlet opening, and entraining the heat softened glass in

the blast whereby the glass is attenuated into fibers by the heat and force of the blast.

4. The process of making glass fibers which comprises burning a combustible mixture of gases within a substantially closed chamber and discharging the burned gases through an opening in one side of the chamber adjacent the bottom wall of the latter in the form of a radially directed blast of a temperature above the attenuating temperature of glass and having a velocity sufficient to attenuate softened glass into fibers, heating a body of glass to a temperature which exceeds the softening point of glass by introducing the body of glass into the burning gases within the chamber, collecting the heat softened glass on the bottom wall of the chamber and subjecting the heat softened glass to the action of centrifugal force, flowing the heat softened glass under the influence of centrifugal force over the bottom wall of the chamber in an outward direction into the outlet opening and into the burned gases discharged as a blast through said outlet opening, separating the heat softened glass into individual radially moving streams as the glass leaves the chamber, and entraining the streams of heat softened glass in the blast whereby the glass is attenuated into fibers by the heat and force of the blast.

5. Apparatus for producing glass fibers comprising a vertical burner having a chamber within which a combustible mixture of gases is burned to provide a temperature within the chamber which exceeds the softening temperature of glass, means for introducing into the chamber a body of glass which is heated by the burning gases in the chamber to a temperature above the softening point of the glass, a bottom wall for the chamber having the peripheral edge spaced below the sides of the chamber to provide an annular outlet opening so proportioned with respect to the volume of the combustion chamber that the burned gases are forced from the chamber in the form of an annular blast having a temperature which exceeds the softening temperature of the glass and having a velocity high enough to draw out the softened glass into fibers, means for rotating the bottom wall at a speed determined to provide the centrifugal force required to flow heat softened glass collected on the bottom wall in a radially outward direction through said outlet opening and into the blast of gases escaping from the chamber.

6. Apparatus for producing glass fibers comprising a burner having a chamber within which a combustible mixture of gases is burned to provide a temperature within the chamber which exceeds the softening temperature of glass, means for introducing into the chamber a body of glass which is heated by the burning gases in the chamber to a temperature above the softening point of the glass, a bottom wall for the chamber having the peripheral edge spaced below the sides of the chamber to provide an annular outlet opening so proportioned with respect to the volume of the combustion chamber that the burned gases are forced from the chamber in the form of an annular blast having a temperature which exceeds the softening temperature of the glass and having a velocity high enough to draw out the softened glass into fibers, means for rotating the bottom wall at a speed determined to provide the centrifugal force required to flow heat softened glass collected on the bottom wall in a radially outward direction

through said outlet opening and into the blast of gases escaping from the chamber, and means at the peripheral edge of said bottom wall for separating the heat softened glass into a multiplicity of individual glass streams.

5. Apparatus for producing glass fibers comprising a burner having a substantially closed chamber within which a combustible mixture of gases is burned to provide a temperature within the chamber which exceeds the softening temperature of glass, means for introducing into the chamber a body of glass which is heated by the burning gases in the chamber to a temperature above the softening point of the glass, a bottom wall for the chamber having the peripheral edge spaced below the sides of the chamber to provide an annular outlet opening so proportioned with respect to the volume of the combustion chamber that the burned gases are forced from the chamber in the form of an annular blast having a temperature which exceeds the softening temperature of the glass and having a velocity high enough to draw out the softened glass into fibers, said bottom wall being shaped to form a well for collecting the heat softened glass, and means for rotating the bottom wall at a speed determined to provide the centrifugal force required to flow heat softened glass in a radially outwardly direction over the bottom wall and through the annular outlet opening into said blast.

20 30 35 40 45 50 55 60 65 70 75 80 85 90 95 100

8. The process of making fibers from a heat softenable material capable of being drawn out into fibers when in a softened state which comprises burning a combustible mixture of gases within a substantially closed chamber and discharging the burned gases from the chamber in the form of a radially directed blast moving at a velocity sufficient to attenuate the heat softened material into fibers, discharging a body of said material in a molten state by centrifugal force into said blast, and entraining the material in the blast whereby the material is attenuated to fibers by the heat and force of the blast.

9. The process of making fibers from a heat softenable material which comprises burning a combustible mixture of gases in a substantially closed chamber and discharging the burned gases from the chamber in the form of an annular radially directed blast moving at a velocity sufficient to attenuate the heat softened material into fibers, subjecting a body of said heat softened material to the action of centrifugal force to flow the material under the influence of the centrifugal force into the blast whereby the material is conveyed from the chamber by the blast, and attenuating the softened material into fibers by the heat and force of the blast.

CHARLES J. STALEGO.  
WENDELL W. DRUMMOND.

#### REFERENCES CITED

The following references are of record in the file of this patent:

#### UNITED STATES PATENTS

| Number       | Name          | Date           |
|--------------|---------------|----------------|
| 2,333,218    | Von Pazsiczky | Nov. 2, 1943   |
| 2,431,205    | Slayer        | Nov. 18, 1947  |
| 2,450,363    | Slayer et al. | Sept. 28, 1948 |
| 70 2,455,907 | Slayer        | Dec. 7, 1948   |

#### FOREIGN PATENTS

| Number     | Country     | Date          |
|------------|-------------|---------------|
| 571,807    | Germany     | Mar. 6, 1933  |
| 75 215,101 | Switzerland | Sept. 1, 1941 |